

G. W. Chapman  
Carpet Lining.

No 80,913.

Patented Aug. 11, 1868.



Witnesses,

J. B. Kidder  
C. Warren Brown

Inventor  
Geo W. Chapman  
by his Atty  
Crosby, Halstead & Fowler

# United States Patent Office.

GEORGE W. CHIPMAN, OF BOSTON, MASSACHUSETTS.

*Letters Patent No. 80,913, dated August 11, 1868.*

## IMPROVEMENT IN CARPET-LINING.

The Schedule referred to in these Letters Patent and making part of the same.

TO ALL WHOM IT MAY CONCERN:

Be it known that I, GEORGE W. CHIPMAN, of Boston, in the county of Suffolk, and State of Massachusetts, have invented an Improvement in Carpet-Lining; and I do hereby declare that the following, taken in connection with the drawings which accompany and form part of this specification, is a description of my invention sufficient to enable those skilled in the art to practise it.

United States Letters Patent, No. 14,585, granted to J. R. Harrington, and now owned by me, relate to the manufacture of a carpet-lining, consisting of a continuous sheet or layer of soft, loose, fibrous material, surfaced by a sheet or sheets of stout paper, the batting being kept in place, relatively to the surface of the paper, by cement or otherwise.

The means for so uniting the paper and wadding have been to cement the entire inner surface of the paper to the wadding, to press the sheets together, to cement together the adjacent edges of the paper sheets, or to stitch the sheets together, each of these means being practicable, though there are some objections to the use of either.

In my present invention I use cementitious matter to confine the sheets together, but instead of spreading it over the whole surface of the paper, I apply it in spots, or in parallel lines, whereby I retain the general elasticity of the wadding, or prevent the paper and wadding from matting together, as they incline to do in covering the paper with cement, and counteract the tendency of the paper to tear at the lines of connection, as it inclines to do in sewed linings.

My invention consists in a carpet-lining, in which the sheets of paper and of soft fibrous filling are secured together, or from relative lateral displacement, by spots or lines of cement, distributed over the surfaces in contact, at such intervals of space as shall permit the lining to preserve the general fulness or elasticity desirable in a carpet-lining.

The drawing represents a piece of carpet-lining embodying my improvement.

*a and b* denote the two sheets of paper; *c*, the soft wadding or batting enclosed between them.

*d* denote spots of cement, or spots opposite to which the cement is applied, the cement being dropped or applied, by a suitable brush, to the inner surface of the paper, at regular intervals, by mechanism connected with and forming part of the lining-making machine, the cement being applied to each sheet of paper just before the paper and wadding come into contact.

Instead of using drops or spots of cement in this manner, the cement may be applied in short lines, as shown at *e*, or in continuous lines, as shown at *f*.

I claim a carpet-lining, the wadding and paper sheets of which are confined together by the lines or spots of cement, substantially as set forth.

GEO. W. CHIPMAN.

Witnesses:

FRANCIS GOULD,  
L. H. LATIMER.